

# UNITED STATES PATENT OFFICE.

JOKICHI TAKAMINE, OF NEW YORK, N. Y., AND JOKICHI TAKAMINE, JR., OF CLIFTON, NEW JERSEY.

## PROCESS OF TREATING TEXTILE AND OTHER FABRICS, THREAD, YARN, AND THE LIKE.

1,421,613.

Specification of Letters Patent. Patented July 4, 1922.

No Drawing.

Application filed October 8, 1920. Serial No. 415,519.

To all whom it may concern:

Be it known that we, JOKICHI TAKAMINE and JOKICHI TAKAMINE, Jr., both subjects of the Emperor of Japan, and residents, respectively, of the city, county and State of New York, and Clifton, county of Passaic, State of New Jersey, have made a certain new and useful Invention in Processes of Treating Textile and Other Fabrics, Thread, Yarn, and the like, of which the following is a specification.

This invention relates to a process of treating textile and other fabrics, yarn, thread and the like.

15 The object of the invention is to provide a process which is simple, economical and efficient for the treatment of textile and other fabrics, yarn, thread and the like, for the removal therefrom of starch, gum 20 and other substances contained therein.

The invention consists substantially in the mode of operation hereinafter set forth and finally pointed out in the claims.

25 It is the common practice in the textile industry to size or starch yarns, thread or the like employed in the manufacture of textile and other fabrics, in order to render the yarn, thread or the like stiffer and harder and more easily manipulated in the textile

30 machinery employed. The result of the sizing of the yarn, thread or the like is that when the fabric is woven therefrom it is saturated or filled with the sizing material. The textile and other fabrics are also ordinarily bleached and dyed to produce the finished product. Before the bleaching and 35 dyeing operations can be properly accomplished, it is necessary to remove the sizing material in order to permit the substances

40 employed to bleach and dye the fabric to penetrate into the body thereof. Various ways of de-sizing have heretofore been employed. One usual method is to treat the yarn, thread or fabric with a fermenting

45 agent, in order that the bacteria of the fermenting agent may act upon the gums and starch content of the materials to be treated, in order to dissolve or decompose the same. For this purpose the yarn, thread, fabric or the like is moistened with water and placed in a vat, and the fermenting agent is then added thereto. After the fermenting operation and the resulting decomposition or dissolution of the gums, starch, etc., from

the yarn, thread or fabric, the latter are 51 washed to remove the dissolved or decomposed gums, starch and other matter.

The great difficulty with this method of 56 treating fabrics, yarns, threads and the like is that it takes too long a period of time, and 60 is not thorough. Frequently a week or longer is required for the fermenting operation, and even then the thorough decomposition or dissolution of the gums, starch and other matter contained in the fabric, 65 yarn, thread or the like is not accomplished.

Another method which has been employed is to subject the fabric, yarn, thread or the like to the action of steam in the presence of an alkali such, for example, as weak caustic soda, soda ash or soaps. This method is objectionable for the reason that, although it is quicker than the method above described, the alkali employed to dissolve or decompose and remove the sizing compound is 70 liable to attack the fibre of the yarn, thread or the like, thereby weakening it or impairing its strength as well as injuriously affecting its luster and other properties.

It has also been proposed to employ malt 80 or malt extract in treating fabrics, but malt products act only on the starchy constituent of the materials to be treated, and do not affect the gums, protein, pectin and other like substances of such materials which, however, it is important to remove. Moreover the action of malt products is slow and large relative quantities are required, which 85 greatly increases the cost of the treatment.

It is among the special purposes of our 90 present invention to avoid the objections above noted, and others, and to provide a method of operation which is economical and expeditious, and wherein the gums, starch and other substances and impurities may 95 be thoroughly removed from the fabrics without danger of impairing the strength of the fibres of the yarn, thread or the like employed in producing the fabric.

In carrying out our invention we propose 100 to employ a substance possessing diastatic and proteolytic properties, and we propose to obtain the substance possessing these properties from a vegetable source, and which substance is economical and expeditious in its action, and thoroughly effective 105 in dissolving and decomposing the starches, gums and the like of the sizing material em-

ployed or contained in the fibres of the yarn, thread or the like, without impairing or weakening such fibres.

In carrying out our invention we employ 5 the seed spores of the microscopic fungi, which are sown on a culture medium, and propagated under suitable conditions of 10 temperature and humidity, for a sufficient period of time for the fungus to attain that stage in which it develops its greatest enzymic power. The enzymic substances contained in the fungus growth are then extracted from the mass or medium upon which 15 the fungus is grown by suitable solvents and manipulation to obtain the enzymic product. The seed spores of the fungi genera Aspergillus Penicillium or Mucor, and particularly the seed spores of the species Eu- 20 rotium Oryzae are suitable for the purpose. The seed spores of other species or genera 25 may likewise be employed, and especially the seed spores of fungi which are capable of being propagated in a fungus growth from which an enzyme is produced which 30 possesses strongly proteolytic power. A fun- 35 gus has been isolated, and to which the name Takochi has been given, which will answer the desired purpose.

A culture medium upon which the fungus 30 seed spores are to be sown and the fungus propagated is prepared, and for this purpose we have found that comminuted or broken grains of cereals such as wheat, corn, oats, barley, etc., and preferably such broken 35 or comminuted grains from cereals from which the greater part of the starchy matter has been removed, leaving the mass in the form of bran, shorts, middlings, etc., and particularly wheat bran, constitute suitable 40 media upon which the fungus may be propagated. Other media may likewise be em- 45 ployed such, for example, as slops from al- cohoilic distillation, residue from beer brew- ing, oil cake, brans, slops and residue from sugar, glucose and starch factories and the like.

The mass to constitute the culture me- 50 dium is first moistened with water and ster- 55 ilized with steam, if desired, and we prefer to add to the mass or medium suitable nour- 60 ishing or fertilizing substances, and for this purpose we have found that glucose, pep- tones, sodium phosphate, sodium chloride, and sodium magnesium salts are excellent. The fertilizing or nourishing substances are 65 thoroughly mixed with the sterilized mass. The fungus seed spores are then sown upon the composition mass, preferably while the latter is in a moistened state, containing 70 from 30 to 60 per cent of moisture. It is not essential that the mass be sterilized, and this operation may be omitted, although we have 75 found that a more abundant and healthy growth of fungus is secured, and a greater 80 development of enzymic power is attained by

first sterilizing the mass. Moreover, in the sterilizing operation, the bacteria contained in the culture medium are more or less de- 70 stroyed or rendered inert, thereby removing the undesirable fermenting or decomposing action thereof, in the resulting enzymic sub- 75 stance to be produced.

After sowing the fungus spores upon the culture medium prepared as above described, the entire mass may be bedded up to a thick- 80 ness of from 6 to 24 inches. Where wheat bran, shorts, middlings, etc., are employed, the bedding up of the culture medium inocu- 85 lated with the fungus spores is not essential. The mass is then maintained in a moist at- 90 mosphere, and at a uniform temperature not to exceed 45 degrees centigrade. In the course of from 8 to 20 hours, the spores be- 95 gin to sprout, and within 20 to 30 hours the growth of the fungus becomes abundant. Carbonic acid gas and heat are evolved dur- 100 ing this period. Within 30 to 60 hours en- 105 zymic properties are developed in the cul- ture medium by the growth of the fungus. This is referred to as a "still growth" method.

Another method of carrying on the propa- 95 gation and development of the fungus growth is to maintain the mass in motion in suitable apparatus or otherwise in such manner as to cause every portion of the inoculated mass to become exposed to the air, thereby preventing the mass from develop- 100 ing too great a heat. Ordinarily the same period of time is required as in the still 105 growth method.

The enzymes produced by the fungus growth are mostly soluble in water, and pos- 110 sess various characteristics such as diastatic, proteolytic, fat splitting, milk coagulating and the like. The relative proportions of 115 these characteristics or properties vary with different species of spores employed, and also to a more or less extent, according to temperature, humidity, method of handling and other conditions observed during the 120 propagation and growth of the fungus.

The various enzymes being soluble in 125 water are easily extracted from the mass upon which the fungus has been grown by lixiviating the mass with water. The solution thus obtained may be employed di- 130 rectly in carrying out our process of treat- ing textile and other fabrics, yarn, thread or the like, or an extract may be concen- trated in any convenient manner. For ex- ample, a desirable degree of concentration may be effected by percolating the semi- aqueous extract or solution through suc- 135 cessive new batches or masses of the culture medium upon which the fungus has been grown.

Of the enzymes contained in this solution thus obtained diastatic enzymes usually pre- 140 dominates followed by proteolytic, milk co-

agulating, fat splitting and others cited in their relative strength.

The solution or extract obtained as described, containing as it does, not only a 5 diastatic but also proteolytic properties, is particularly useful in the textile industry for de-sizing and de-gumming textile and other fabrics, such as silk, cotton, etc., ramie, China grass or other fibre, yarn, thread and 10 the like, the diastatic property of the solution being employed to dissolve the starch content of the sizing material employed, and the proteolytic power of the extract or solution being utilized to dissolve the gums. 15 To render the extract or solution stable, and to enable it to be maintained without material deterioration, we employ the joint effect of heat and an antiseptic, being careful to avoid the use of a sufficient degree of 20 heat to impair the enzymic power of the solution, and also to employ an antiseptic in insufficient quantity to injure or impair the enzymic power of the extract. We have found that a temperature of 45 degrees, and 25 an antiseptic, for example sulphurous acid, in the preparation of one part to from 1 to 10,000 parts of the enzymic substance, supply the necessary conjoint effective action to render the solution stable, whereas neither 30 the heat nor the antiseptic alone will answer the purpose.

Other antiseptics may be employed, such as phenol, creosol, or other coal tar derivatives, or formaldehyde.

35 Where the enzymic solution is to be employed immediately after obtaining it, it becomes unnecessary to subject the same to the action of heat and a preservative.

To effect the de-sizing and de-gumming of 40 the textile or other fabric, yarn, thread or the like, the material to be treated is immersed in a weak aqueous solution of the enzymic extract, and permitted to stand for several hours. We have found from 6 to 10 45 hours ordinarily is sufficient. During this period the enzymes act upon the starch and gum contents of the material to render the same soluble and easily washed way, without attacking, weakening or otherwise impairing the fibres of the material, leaving the 50 same clean and free from starch or gum substances. The material to be treated is then washed in water in order to remove the dissolved gums and starch, and such material is 55 then ready for the bleaching and dyeing operations.

By reason of the fibres of the material being thus rendered clean and free from sizing material, gums and the like, they more easily 60 and readily respond to the bleaching material and absorb the dyes, which are thus permitted to penetrate more thoroughly into the bodies of the fibres.

In the case of yarn, thread or the like, 65 after the treatment with the extract solution,

where no bleaching or dyeing is required, or after such treatment and the bleaching and dyeing operations, where the latter are required, they are woven into textile fabrics in the regular way.

The process of our invention effects a more thorough and complete de-sizing and de-gumming action than is possible with the methods and processes heretofore used, and is more expeditious than such prior methods. 70 It also dispenses in the case of silk fabrics, for instance, with the use of soap alkali, and which is likely to cause injury to the silk fibres. In the case of silk waste, a by-product of silk weaving, the silk fibres become 75 stuck together by the gums content, making it almost a solid and unworkable mass. The enzymic substance digests or dissolves these gums thereby rendering the fibre contained in such waste clean and usable for weaving 80 into silk fabrics.

In the case of ramie fibre, China grass and like vegetable materials, the starch and gums contained therein are easily removed without impairment of the fibre by the use of an 90 enzymic substance in accordance with our invention, thus rendering it unnecessary to employ for this purpose soda or soaps.

It is understood, of course, that our invention is equally well adapted for use in the 95 treatment of fibres, yarn, thread or the like before being woven into fabrics, as well as in connection with fabrics after having been woven. We do not desire, therefore, to be limited or restricted in this connection.

Having now set forth the objects and nature of our invention and the method of carrying the same into practical operation, what we claim as new and useful, and of our own invention, and desire to secure by Letters 100 Patent is:

1. The process of treating textiles for the removal therefrom of starches, gums and other substances, which comprises subjecting the textile to a bath containing proteolytic and diastatic enzymes, and permitting said enzymes to act on said substances to dissolve the same, and then washing the textile in water.

2. The process of de-sizing and de-gumming textile and other fabrics, thread, yarn and the like, which comprises subjecting the same to the action of an antiseptic enzymic substance of vegetable fungus origin.

3. The process of de-sizing and de-gumming textile and other fabrics, thread, yarn and the like, which comprises subjecting the same to a stable liquid containing diastatic and proteolytic enzymes of vegetable origin.

4. The process of treating textiles for the removal therefrom of starches, gums and other substances, which comprises subjecting the textile to a bath containing an aqueous solution of proteolytic and diastatic en-

- zymes of vegetable fungus origin to render soluble said substances, and then washing the textile in water to remove the solubilized substances.
5. The process of de-sizing and de-gumming textile and other fabrics, thread, yarn and the like, which comprises treating the same with an aqueous extract containing diastatic and proteolytic enzymes of vegetable origin and possessing properties whereby water-insoluble substances of said fabrics are rendered soluble and capable of being washed out with water.
6. The process of de-sizing and de-gumming textile and other fabrics, thread, yarn and the like, which comprises treating the same with an aqueous extract containing diastatic and proteolytic enzymes of vegetable origin, and then washing the same in water.
7. The process which comprises solubilizing the starches, gums and other substances contained in textiles with an enzyme of vegetable fungus origin possessing proteolytic and diastatic properties, and then washing the textile in water to remove the solubilized substances.
8. The process of treating textile and other fabrics, thread, yarn or the like, for the removal of soluble substances therefrom, which comprises rendering soluble such substances with a material containing diastatic and proteolytic enzymes of vegetable origin, and then washing the fabric, thread, yarn or the like to remove the soluble substances therefrom.
9. The process which comprises propagating a vegetable fungus upon a culture medium to develop diastatic and proteolytic properties therein, then rendering soluble or decomposing the starchy and gummy substances contained in fabrics, thread, yarn or the like, with such diastatic and proteolytic substances, and finally washing such fabric, thread, yarn or the like with water. 40
10. The process which comprises propagating a vegetable fungus upon a culture medium to develop diastatic and proteolytic properties therein, then extracting the diastatic and proteolytic properties from the culture medium, and then stabilizing said extract for use in rendering soluble the starchy and gummy substances contained in fabrics, thread, yarn or the like, with such extract. 50
11. The process which comprises propagating a vegetable fungus upon a culture medium to develop diastatic and proteolytic properties therein, then extracting the diastatic and proteolytic properties from the culture medium, and then subjecting said extract to a stabilizing temperature and antiseptic and thereafter subjecting the starchy and gummy substances contained in fabrics, thread, yarn or the like, with such extract, and finally washing the fabric, thread, yarn or the like with water. 60

In testimony whereof we have hereunto set our hands on this 30th day of September, A. D. 1920.

JOKICHI TAKAMINE.  
JOKICHI TAKAMINE, JR.